

# UNITED STATES PATENT OFFICE.

FRANK COCHRANE, OF CHEADLE HULME, ENGLAND.

## PRODUCTION OF FABRICS HAVING THE PROPERTY OF INVISIBILITY.

1,306,213.

Specification of Letters Patent. Patented June 10, 1919.

No Drawing.

Application filed June 18, 1917. Serial No. 175,522.

To all whom it may concern:

Be it known that I, FRANK COCHRANE, a subject of the King of Great Britain and Ireland, and resident of Middleton Cottage, 5 Cheadle Hulme, in the county of Chester, England, have invented certain new and useful Improvements Relating to the Production of Fabrics Having the Property of Invisibility, of which the following is a 10 specification.

This invention relates to the production of fabrics which, by their coloring, are given a high degree of invisibility when looked at from a distance, and has for its object to 15 provide an effective and ready method of producing such fabrics.

My invention comprises the padding of the fabric with a solution of a coloring matter capable of producing at least two 20 colors by development by suitable metallic salts, and the development and fixing (by treatment with one metallic salt) of a uniform ground color upon which the other color or colors is or are developed in 25 promiscuous patches by the application of other metallic salts by hand or otherwise.

In one convenient application of my invention, the cotton, woolen, linen or other fabric is padded in a cold solution of suitable 30 dyewood extracts such as fustic, cutch and sumac. It is then passed through a bath of a boiling aluminium salt, whereby the ground color, such as fustic, is developed and fixed.

35 Other developers or metallic salts, such as potassium bichromate, and suitable salts of iron, are applied by hand or otherwise to produce promiscuous color patches. The fabric is then folded and allowed to stand 40 so that the colors may spread and blend with the ground color and also so that the metallic salts on contacting parts of the material may print off or transfer from one to the other. The fabric is then dried at a 45 high temperature in order to further develop and fix the colors.

The aluminium salt employed in the developing and fixing of the ground color acts as a retarder upon the subsequent metallic salts so that the colors produced are less pronounced and blend with or shade off into the ground better than they otherwise would.

The dyewood extracts and metallic salts

hereinbefore specified are employed in solutions of the concentrations usual in processes of dyeing with said materials.

In another convenient application of my invention, I fix a suitable mordant (such as aluminium acetate or tin chlorid) upon the fabric and then pass the latter through a dye solution comprising coloring matter or media (such as fustic, cutch and sumac) for producing a plurality of colors, one color *i. e.*, the ground color, being developed by the mordant aforesaid and the remaining colors being ready for subsequent development in promiscuous patches in a manner substantially as in connection with the previously described application of my invention.

Having now described my invention what I claim as new and desire to secure by Letters Patent is:—

1. The process of producing fabrics having the property of invisibility consisting in padding the fabric in a solution of a coloring matter capable of producing a plurality of colors by development by metallic salts, developing and fixing a uniform ground color by one metallic salt and developing and fixing promiscuous color patches upon said ground color by at least one other metallic salt, as set forth.

2. In the production of fabrics having the property of invisibility, the treatment of the fabric as follows:—(1) Padding the fabric with a solution of a coloring matter capable of producing a plurality of colors by development by means of metallic salts (2) developing and fixing a uniform ground color by treatment with one metallic salt (3) developing upon the ground color promiscuous color patches in a plurality of colors by the application of a plurality of separate metallic salts by hand, as set forth.

3. In the production of fabrics having the property of invisibility, the treatment of the fabric as follows:—(1) Padding in a cold solution of dyewood extracts (2) developing and fixing a uniform ground color by a metallic salt (3) developing upon the ground color a plurality of other colors in promiscuous patches by the application of other metallic salts by hand (4) drying the fabric at a high temperature, as set forth.

4. In the production of fabrics having the property of invisibility, the treatment

of the fabric as follows:—(1) Padding in a cold solution of fustic, cutch and sumac (2) developing and fixing a uniform ground by passing the fabric through a bath of boiling aluminium salt (3) developing upon the ground color a plurality of other colors in promiscuous patches by the application of potassium bichromate and suitable salts of iron by hand (4) folding the wet fabric

(5) drying the fabric at a high temperature, 10 as set forth.

In testimony whereof I have signed my name to this specification in the presence of two subscribing witnesses.

FRANK COCHRANE.

Witnesses:

ARTHUR HUGHES,  
EWALD SIMPSON MOSELEY.

Copies of this patent may be obtained for five cents each, by addressing the "Commissioner of Patents, Washington, D. C."